

1

2,974,037

**HIGH TEMPERATURE COBALT BASE ALLOY**

Rudolf H. Thielemann, Palo Alto, Calif., assignor to Sierra Metals Corporation, Chicago, Ill., a corporation of Delaware

No Drawing. Filed July 28, 1958, Ser. No. 751,162

8 Claims. (Cl. 75—171)

This invention relates to a cobalt base metal alloy, which includes alloying metal additives which make the resulting alloy corrosion resistant and of great mechanical work strength at temperatures up to as high as 1800° F.

Important features of the alloy of this invention are that it may be cast, is highly resistant to oxidation and other forms of corrosion at temperatures up to about 1800° F., and possesses great mechanical work strength at temperatures up to between 1500° F. and 1800° F. As a result, this alloy may be used in the manufacture of blades, vanes, and other parts of high temperature gas turbine engines. Other important uses of the alloy of this invention are in the manufacture of exhaust valves and manifolds in internal combustion engines, in heat exchangers, and in linings for retorts and container vessels used in the chemical and metallurgical industries.

The prior art nickel and/or cobalt base metal alloys which have been used as blades, vanes, and other parts of high temperature gas turbine engines, have a maximum operating temperature of about 1500° F. For example, a common nickel-cobalt base metal alloy which incorporates molybdenum as a constituent is for all practical purposes non-utilizable as a structural member in a gas turbine engine if the metal temperature is above 1500° F. The oxidation resistance of such an alloy fails above 1500° F.

Since the alloy of this invention used in blades or vanes in a high temperature gas turbine engine is corrosion resistant and has higher tensile strength at markedly higher temperatures than conventional alloys, the gas turbine engine can be operated at such higher temperature. The performance of the gas turbine engine is improved, in that the total thrust is increased and the amount of fuel consumed per pound of thrust is decreased.

The metal alloy of this invention is comprised by weight of approximately: 15 to 30 percent of chromium; 5 to 15 percent of tungsten; from 0.5 to 5 percent of columbium; from 0.1 to 1.3 percent of carbon; from 0.01 to 0.2 percent of boron; and the balance, essentially cobalt.

I have found that the strength characteristics of the alloy of this invention are improved by the addition of the boron, as specified, in an amount of from about 0.01 percent up to about 0.2 percent. The addition of this constituent in the amounts specified improves the high temperature metallurgical stability and the strength characteristics of the alloy of this invention. However, if the boron content exceeds 0.2 percent, then the alloy of this invention may be unsatisfactory, particularly in those applications where thermal shock requirements are important.

Tantalum may be present in an amount such that if the amount of columbium in the alloy is greater than 3 percent, the combined amount of tantalum and columbium is less than or equal to 20 percent of the alloy, and if the amount of columbium in the alloy is equal

2

to or less than 3 percent, then the tantalum should never exceed twice the amount of columbium in the alloy.

Molybdenum may be tolerated in the alloy of this invention without deleteriously affecting the properties of the alloy, provided the amount of molybdenum in the alloy is not more than one-half the amount of tungsten in the alloy, and in any event, is no greater than 3.5 percent by weight of the alloy.

While silicon, nickel and iron are not essential ingredients to the metal alloy of the present invention, it has been found that the addition of small percentages of any one or more of these ingredients, that is, up to about 1.5 percent of silicon, and up to about 5 percent of nickel and/or iron may in certain cases somewhat improve the oxidation resistance of the alloy.

An alloy having the above composition is particularly resistant to oxidation and has high strength at elevated temperatures above 1500° F., so as to be suitable for use in forming cast liners for retorts and container vessels used in the chemical and metallurgical industries as well as for blades or vanes in high temperature gas turbine engines.

To achieve the optimum desired properties, it is preferred that the following impurities in the alloy be held to the following limits by weight. The manganese content in the final alloy should be no more than about 2 percent. The interstitial elements such as nitrogen, hydrogen, tin, lead and the like should be kept as low as possible. In addition, no more than about 0.5 percent total of deoxidizers such as calcium, magnesium and the like should be present.

Following are examples of the preparation and test results of the cobalt base metal alloy of this invention.

**Example 1**

A 5 pound alloy melt of a cobalt base metal alloy composition containing about 20 percent of chromium, about 10 percent of tungsten, about 1.4 percent of columbium, about 0.01 percent of boron, about 0.55 percent of carbon, and the balance, substantially all cobalt, all by weight, was prepared by melting a chromium-cobalt mix in a magnesia crucible under high vacuum conditions, following which the tungsten, columbium, boron and carbon in the form of graphite were added.

A cluster of 6 test bars were formed from the 5 pound melted alloy heat by the usual investment casting technique under high vacuum conditions. These bars were each 3 inches long and  $\frac{1}{4}$  inch in diameter.

The test bars had an elongation of about 5.5 percent at room temperature under a tensile stress of 110,000 p.s.i.

The test bars of this example had a rupture life in excess of 100 hours under a load of 25,000 p.s.i. at a temperature of 1600° F. in air; and a rupture life in excess of 100 hours under a load of 20,000 p.s.i. at a temperature of 1700° F. in air.

**Example 2**

A 5 pound alloy melt and test bars of the same dimensions as set forth in Example 1 of a cobalt base metal alloy composition containing about 20 percent of chromium, about 10 percent of tungsten, about 1 percent of tantalum, about .5 percent of columbium, about 0.01 percent of boron, about 0.5 percent of carbon, and the balance, essentially cobalt, all by weight, were prepared in the same manner as set forth in Example 1.

The test bars of this example had an elongation of 6.5 percent at room temperature under a tensile stress of 95,000 p.s.i.

The test bars of this example had a rupture life in excess of 100 hours under a load of 20,000 p.s.i. at a temperature of about 1600° F. in air; and a rupture life



metal alloy composition containing about 23 percent of chromium, about 7 percent of tungsten, about 5 percent of tantalum, about 5 percent of columbium, about 0.01 percent of boron, about 1.3 percent of carbon, and the balance, essentially cobalt, all by weight, were prepared in the same manner as set forth in Example 1.

The test bars of this example had an elongation of 2 percent at room temperature under a tensile stress of 115,000 p.s.i.

The test bars of this example had a rupture life in excess of 100 hours under a load of 20,000 p.s.i. at a temperature of about 1600° F. in air and a rupture life in excess of 100 hours under a load of 15,000 p.s.i. at a temperature of about 1700° F. in air.

*Example 12*

A 5 pound alloy melt and test bars of the same dimensions as set forth in Example 1 of a cobalt base metal alloy composition containing about 30 percent of chromium, about 5 percent of tungsten, about 5 percent of tantalum, about 3 percent of columbium, about 2.5 percent of molybdenum, about 0.01 percent of boron, about 0.3 percent of carbon, and the balance, essentially cobalt, all by weight, were prepared in the same manner as set forth in Example 1.

The test bars of this example had an elongation of about 8.5 percent at room temperature under a tensile stress of 100,000 p.s.i.

The test bars of this example had a rupture life in excess of 100 hours under a load of 18,000 p.s.i. at a temperature of about 1600° F. in air, and a rupture life in excess of 100 hours under a load of 12,000 p.s.i. at a temperature of about 1700° F. in air.

*Example 13*

A 5 pound alloy melt and test bars of the same dimensions as set forth in Example 1 of a cobalt base metal alloy composition containing about 18 percent of chromium, about 8.6 percent of tungsten, about 3.5 percent of tantalum, about 3.5 percent of columbium, about 3.5 percent of molybdenum, about 0.1 percent of boron, about 0.5 percent of carbon, and the balance, essentially cobalt, all by weight, were prepared in the same manner as set forth in Example 1.

The test bars of this example had an elongation of 4 percent at room temperature under a tensile stress of 100,000 p.s.i.

The test bars of this example had a rupture life in excess of 100 hours under a load of 20,000 p.s.i. at a temperature of about 1600° F. in air and a rupture life in excess of 100 hours under a load of 15,000 p.s.i. at a temperature of about 1700° F. in air.

*Example 14*

A 5 pound alloy melt and test bars of the same dimensions as set forth in Example 1 of a cobalt base metal alloy composition containing about 23 percent of chromium, about 5 percent of tungsten, about 5 percent of tantalum, about 3 percent of columbium, about 2.5 percent of molybdenum, about 0.01 percent of boron, about 0.3 percent of carbon, about 1.5 percent of silicon, about 2.5 percent of nickel, about 2.5 percent of iron, and the balance, essentially cobalt, all by weight, were prepared in the same manner as set forth in Example 1.

The test bars of this example had an elongation of about 2 percent at room temperature under a tensile stress of 95,000 p.s.i.

The test bars of this example had a rupture life in excess of 100 hours under a load of 20,000 p.s.i. at a temperature of about 1600° F. in air and a rupture life in excess of 100 hours under a load of 15,000 p.s.i. at a temperature of about 1700° F. in air.

*Example 15*

A 5 pound alloy melt and test bars of the same di-

mensions as set forth in Example 1 of a cobalt base metal alloy composition containing about 20 percent of chromium, about 10 percent of tungsten, about 1.4 percent of columbium, about 0.01 percent of boron, about 0.55 percent of carbon, about 0.2 percent of silicon, about 1.0 percent of nickel, about 1.0 percent of iron, and the balance, essentially cobalt, all by weight, were prepared in the same manner as set forth in Example 1.

The test bars of this example had an elongation of about 6 percent at room temperature under a tensile stress of 110,000 p.s.i.

The test bars of this example had a rupture life in excess of 100 hours under a load of 20,000 p.s.i. at a temperature of about 1600° F. in air, and a rupture life in excess of 100 hours under a load of 15,000 p.s.i. at a temperature of about 1700° F. in air.

*Example 16*

A 5 pound alloy melt and test bars of the same dimensions as set forth in Example 1 of a cobalt base metal alloy composition containing about 20 percent of chromium, about 7.5 percent of tungsten, about 2.5 percent of tantalum, about 2.0 percent of columbium, about 0.01 percent of boron, about 0.5 percent of carbon, about 0.1 percent of silicon, about 1.5 percent of nickel, about 1.5 percent of iron, and the balance, essentially cobalt, all by weight, were prepared in the same manner as set forth in Example 1.

The test bars of this example had an elongation of about 4 percent at room temperature under a tensile stress of 100,000 p.s.i.

The test bars of this example had a rupture life in excess of 100 hours under a load of 20,000 p.s.i. at a temperature of about 1600° F. in air and a rupture life in excess of 100 hours under a load of 15,000 p.s.i. at a temperature of about 1700° F. in air.

*Example 17*

A 5 pound alloy melt and test bars of the same dimensions as set forth in Example 1 of a cobalt base metal alloy composition containing about 15 percent of chromium, about 15 percent of tungsten, about 2 percent of tantalum, about 2.5 percent of columbium, about 0.01 percent of boron, about 0.65 percent of carbon, about 0.1 percent of silicon, about 0.5 percent of nickel, about 0.5 percent of iron, and the balance, essentially cobalt, all by weight, were prepared in the same manner as set forth in Example 1.

The test bars of this example had an elongation of about 5 percent at room temperature under a tensile stress of 110,000 p.s.i.

The test bars of this example had a rupture life in excess of 100 hours under a load of 20,000 p.s.i. at a temperature of about 1600° F. in air, and a rupture life in excess of 100 hours under a load of 15,000 p.s.i. at a temperature of about 1700° F. in air.

The above detailed description of this invention has been given for clarity of understanding only. No unnecessary limitations should be understood therefrom, as modifications will be obvious to those skilled in the art.

This application is a continuation-in-part of my co-pending United States application, Serial No. 683,457, filed September 12, 1957, now abandoned.

I claim:

1. A metal alloy consisting essentially of by weight: from about 15 to about 30 percent of chromium; from about 5 to about 15 percent of tungsten; from about 0.01 to about 0.2 percent of boron; from about 0.5 to about 5 percent of columbium; from about 0.1 to about 1.3 percent of carbon; and the balance cobalt.

2. A metal alloy consisting essentially of by weight: from about 15 to about 30 percent of chromium; from about 5 to about 15 percent of tungsten; from about 0.5 to about 5 percent of columbium; tantalum in an amount such that if the amount of columbium in the alloy is

more than about 3 percent, the combined amount of tantalum and columbium is less than or equal to 20 percent of the alloy, and if the amount of columbium in the alloy is equal to or less than about 3 percent, the amount of tantalum being never more than about twice the amount of columbium in the alloy; from about 0.01 to about 0.2 percent of boron; from about 0.1 to about 1.3 percent of carbon, and the balance cobalt.

3. A metal alloy consisting essentially of by weight: from about 15 to about 30 percent of chromium; from about 5 to about 15 percent of tungsten; from about 0.5 to about 5 percent of columbium; up to about 3.5 percent of molybdenum, but not more than about 50 percent of the tungsten present in the alloy; from about 0.01 to about 0.2 percent of boron; from about 0.1 to about 1.3 percent of carbon; and the balance cobalt.

4. A metal alloy consisting essentially of by weight: from about 15 to about 30 percent of chromium; from about 5 to about 15 percent of tungsten; from about 0.5 to about 5 percent of columbium; tantalum in an amount such that if the amount of columbium in the alloy is more than about 3 percent, the combined amount of tantalum and columbium in the alloy is less than or equal to 20 percent of the alloy; and if the amount of columbium in the alloy is equal to or less than about 3 percent, the amount of tantalum being never more than about twice the amount of columbium in the alloy; up to about 3.5 percent of molybdenum, but not more than about 50 percent of the tungsten present in the alloy; from about 0.01 to about 0.2 percent of boron; from about 0.1 to about 1.3 percent of carbon; and the balance cobalt.

5. A metal alloy consisting essentially of by weight: from about 15 to about 30 percent of chromium; from about 5 to about 15 percent of tungsten; from about 0.01 to about 0.2 percent of boron; from about 0.5 to about 5 percent of columbium; from about 0.1 to about 1.3 percent of carbon; up to about 1.5 percent of silicon; up to about 5 percent of nickel; up to about 5 percent of iron; and the balance cobalt.

6. A metal alloy consisting essentially of by weight: from about 15 to about 30 percent of chromium; from about 5 to about 15 percent of tungsten; from about 0.5 to about 5 percent of columbium; tantalum in an amount such that if the amount of columbium in the alloy is more than about 3 percent, the combined amount of tantalum and columbium in the alloy is less than or equal to 20 percent of the alloy, and if the amount of columbium in the alloy is equal to or less than about 3 percent, the amount of tantalum being never more than about twice the amount of columbium in the alloy; up

to about 1.5 percent of silicon; up to about 5 percent of nickel; up to about 5 percent of iron; from about 0.01 to about 0.2 percent of boron; from about 0.1 to about 1.3 percent of carbon; and the balance cobalt.

5 7. A metal alloy consisting essentially of by weight: from about 15 to about 30 percent of chromium; from about 5 to about 15 percent of tungsten; from about 0.5 to about 5 percent of columbium; up to about 3.5 percent of molybdenum, but not more than about 50

10 percent of the tungsten present in the alloy; up to about 1.5 percent of silicon; up to about 5 percent of nickel; up to about 5 percent of iron; from about 0.01 to about 0.2 percent of boron; from about 0.1 to about 1.3 percent of carbon; and the balance cobalt.

15 8. A metal alloy consisting essentially of by weight: from about 15 to about 30 percent of chromium; from about 5 to about 15 percent of tungsten; from about 0.5 to about 5 percent of columbium; tantalum in an amount such that if the amount of columbium in the alloy is

20 more than about 3 percent, the combined amount of tantalum and columbium in the alloy is less than or equal to 20 percent of the alloy, and if the amount of columbium in the alloy is equal to or less than about 3 percent, the amount of tantalum being never more

25 than about twice the amount of columbium in the alloy; up to about 3.5 percent of molybdenum, but not more than about 50 percent of the tungsten present in the alloy; up to about 1.5 percent of silicon; up to about 5 percent of nickel; up to about 5 percent of iron; from

30 about 0.01 to about 0.2 percent of boron; from about 0.1 to about 1.3 percent of carbon; and the balance cobalt.

#### References Cited in the file of this patent

##### UNITED STATES PATENTS

|    |           |                   |               |
|----|-----------|-------------------|---------------|
| 35 | 2,247,643 | Rohn et al. ----- | July 1, 1941  |
|    | 2,486,576 | Savage -----      | Nov. 1, 1949  |
|    | 2,515,774 | Johnson -----     | July 18, 1950 |
| 40 | 2,684,299 | Binder -----      | July 20, 1954 |
|    | 2,771,360 | Malcolm -----     | Nov. 20, 1956 |
|    | 2,855,295 | Hansel -----      | Oct. 7, 1958  |

##### FOREIGN PATENTS

|    |         |                     |               |
|----|---------|---------------------|---------------|
| 45 | 443,821 | Great Britain ----- | Mar. 6, 1936  |
|    | 686,180 | Great Britain ----- | Jan. 21, 1953 |
|    | 542,813 | Canada -----        | June 25, 1957 |

##### OTHER REFERENCES

|    |                                                              |
|----|--------------------------------------------------------------|
| 50 | Materials and Methods, September 1953, Number 260, page 139. |
|----|--------------------------------------------------------------|

UNITED STATES PATENT OFFICE  
CERTIFICATION OF CORRECTION

March 7, 1961

Patent No. 2,974,037

Rudolf H. Thielemann

It is hereby certified that error appears in the above numbered patent requiring correction and that the said Letters Patent should read as corrected below.

In the grant, line 1, name of inventor, for "Rudolph H. Thielemann" read -- Rudolf H. Thielemann --; column 4, line 66, for "85,00 p.s.i." read -- 85,000 p.s.i. --; column 5, line 24, for "prapared" read -- prepared --.

Signed and sealed this 25th day of July 1961.

(SEAL)

Attest:

ERNEST W. SWIDER

Attesting Officer

DAVID L. LADD  
Commissioner of Patents